

June 1, 1926.

1,586,674

E. HÄRTEL

PROCESS OF MANUFACTURING STABLE PAVEMENTS

Filed July 26, 1922



*Inventor*  
*Emil Härtel*

## UNITED STATES PATENT OFFICE.

EMIL HÄRTEL, OF COSWIG, GERMANY.

## PROCESS OF MANUFACTURING STABLE PAVEMENTS.

Application filed July 26, 1922, Serial No. 577,706, and in Germany November 22, 1921.

The object of my invention is to furnish a practical and durable stable pavement, and it consists of two layers, of an isolating, elastic lower layer made of impregnated, 5 crushed cork and a water-shedding, acid- and alkali-proof upper layer which offers a firm foothold to the animals and which, when laying it, is provided with a molten adhesive substance of the same kind as the 10 upper layer for the purpose of producing a homogeneous pavement without joints, a pavement, which, owing to the highly dis- 15 infecting and germ-killing upper layer and the perfect absence of joints, prevents any formation of disease germs and putrefac- 20 tion.

The accompanying drawing shows a perspective view of a pavement made according to my invention. 25 The pavement described above is made in blocks, plates or slabs of varying sizes, as may be most desirable in any particular case. The substance serving as upper layer for the individual slabs and as uniting adhesive medium for them is made of molten mineral and brown coal bitumen, tar, asphaltum, the residues of petrol and suitable benzol derivates, of impregnating oils (creosote and anthracene oil), of disinfecting 30 oils (phenol and crude cresol), while adding crushed natural cork, cork bark, sawdust and chips of wood which are thoroughly mixed in stirring apparatus and after being put on top of the still hot lower 35 slabs are united with them by pressing to one plate or slab.

The substances named, like benzol derivates, residues of petrol, and tar serve not only as uniting and adhesive media but 40 also as germicides. To intensify their well-known effect creosote or benzol derivates like carbolic acid etc. may be mixed with them.

In addition, the substances mentioned 45 have water-shedding properties and cause permanent dryness of the pavement.

By uniting cork barks, sawdust and chips of wood with the bituminous molten mass, as described above, a pavement is produced 50 which in practical use gradually becomes rough and perfectly eliminates the much feared smoothness of asphalt-like substances with the result that the animals are sure-footed when standing or walking.

55 Furthermore, the use of these united slabs

effects an essential saving in laying the pavement as compared with all other kinds of stable pavements put on in layers on the spot or stamped; when laying the latter kinds of stable pavements expensive trans- 60 portations of boilers, kettles, etc. are necessary in addition to the cost of laying, while the slabs described above may be laid by any unskilled person.

The process of manufacturing my isolat- 65 ing stable pavement is as follows: at first impregnated, i. e. water-shedding cork plates are made which form an isolating lower layer. These cork plates, when still hot, are united by pressing them with a 70 molten mass of mineral coal bitumen, brown coal bitumen, coal tar pitch, slag-containing brown coal pitch, natural asphalt mastic, tar, petrol residues, creosote and anthracene oil, cresol (carbolic oil), powdered bark, 75 chips of wood, powdered cork and crushed cork so as to produce perfectly uniform slabs combining the two layers. It is self- 80 evident that the mass for the upper layer must be previously made ready and thor- 85oughly mixed in stirring apparatus. When uniting by pressing the cork plates forming the lower layer with the mass for the upper layer grooves may be pressed into the latter by using a suitable type of press.

Exactly the same mass which forms the 90 upper layer, by varying the quantities of the ingredients added, is worked into a cementing medium which can easily be molten on the spot where the slabs are to be laid and put on the adjoining edges of the slabs. Thus, by joining the slabs together after 95 being treated with the cementing medium a homogeneous pavement without joints is produced which is especially suited for stables, as it is warm, disinfecting, germ- 100 killing, watertight, water-shedding, acid- and alkali-proof, elastic, absolutely imper- 105 meable to humidity or cold from below, and antiseptic.

I am aware that prior to my invention pavements have been made which consist of two layers, f. i. of a lower layer or sub- 110 bed of concrete or artificial stone and an upper layer or wearing surface of cork waste united to the sub-bed by means of tar or similar cementing media. Bricks or blocks of the material named are also known as is the method of placing these blocks or bricks on a sub-bed of cement, while my in-

vention consists in uniting and combining two layers within each individual slab or plate.

Having thus described my invention, 5 what I claim as new, and desire to secure by Letters Patent, is:

1. A pavement for stable-floors herein described, and consisting of individual slabs or plates which constitute a perfect union 10 of two layers viz, of a lower one consisting of a mixture of cork and cementing media and an upper one containing fine cork powder, sawdust, chips of wood, and slag, and, as cementing medium, a mixture of molten mineral and brown coal bitumen or equivalent covering; and a cementing medium for 15 the joints of the said slabs or plates consisting of a mixture of fine cork powder, sawdust, chips of wood, slag, molten mineral and brown coal bitumen or equivalent ingredients.
2. A pavement for stable-floors herein de-

scribed, and consisting of individual slabs or plates which constitute a perfect union 20 of two layers viz, of a lower one consisting of a mixture of cork and cementing media and an upper one containing fine cork powder, sawdust, chips of wood, and slag, and, as cementing medium, a mixture of molten mineral and brown coal bitumen or equivalent covering; and a cementing medium for 25 the joints of the said slabs or plates consisting of a mixture of fine cork powder, sawdust, chips of wood, slag, molten mineral and brown coal bitumen or equivalent ingredients.

In testimony whereof I affix my signature.

EMIL HÄRTEL.